

B. P. HAZELTINE:  
METHOD OF AND MEANS FOR PREVENTING OXIDATION OF ROLLED MATERIAL.  
APPLICATION FILED OCT. 5, 1916.

1,295,986.

Patented Mar. 4, 1919.



Witnesses

Ed. C. Johnson  
67 Murray

Inventor  
B. P. Hazelton

By C. C. Letherman  
Atty.

# UNITED STATES PATENT OFFICE.

BENJAMIN P. HAZELTINE, OF WHEELING, WEST VIRGINIA, ASSIGNOR TO NATIONAL TUBE COMPANY, OF PITTSBURGH, PENNSYLVANIA, A CORPORATION OF NEW JERSEY.

## METHOD OF AND MEANS FOR PREVENTING OXIDATION OF ROLLED MATERIAL.

1,295,986.

Specification of Letters Patent.

Patented Mar. 4, 1919.

Application filed October 5, 1916. Serial No. 123,875.

To all whom it may concern:

Be it known that I, BENJAMIN P. HAZELTINE, a citizen of the United States, and resident of Wheeling, in the county of Ohio 5 and State of West Virginia, have invented certain new and useful Improvements in Methods of and Means for Preventing Oxidation of Rolled Material, of which the following is a specification.

10 My invention relates to the manufacture of steel and has particular reference to an improvement in a method of and means for preventing oxidation of metal flats and similar rolled metal shapes.

15 The desirability of some such method and means has been heretofore recognized and patents have been granted on devices having this desirable object in view. For instance, the patent to Daniels, No. 1,108,144, of August 25, 1914, discloses a method and apparatus, the idea disclosed in that patent being that of immersing the rolled material in water after passing the finishing rolls.

20 My improvement has material advantages over that disclosed in any prior patent in that it provides for the production of an unoxidized material by the use of a much more readily handled medium and the use of a simpler and more economical mechanism. 25 My invention contemplates the employment of a closed passageway for the rolled material from the planishing or finishing rolls, together with means for injecting at suitable intervals a quantity of a 30 gas or vapor in quantities sufficient to prevent oxidation and to gradually cool the material to such extent that it will not oxidize upon being brought into contact with the air after emerging from the closed 35 passageway.

The advantages in the use of such construction arise from the fact that a much more economical mechanism may be employed inasmuch as the problem of leakage 40 of the cooling non-oxidizing medium is not to be considered. The passageway may have open ends at the entrance and exit points, atmospheric air being prevented from entering, due to the excess pressure of the medium employed as the non-oxidizing agent.

45 The method and the means employed in carrying out the same will be better under-

stood by reference to the accompanying drawings, wherein—

Figure 1 is a side elevation somewhat diagrammatic in form showing a mill adapted to carry out my invention; 55

Fig. 2 is an enlarged longitudinal section showing the container or passageway and some of the rolls employed, and 60

Fig. 3 is a sectional view on the line 3—3 of Fig. 2.

Referring more particularly to the drawings, it will be seen that the material is caused to enter the mill over the rollers 10; 65 it passes through the rolls in the stand 11, thence to the repeater 12 and back between the planishing rolls 13. After leaving the planishing rolls, the material enters the conduit 14 at the open end 15. This conduit, 70 as best shown in Fig. 3, may be in the form of a trough having a flat floor along which the material which is indicated at 16 is caused to travel. Feed-out pinch rollers 17 serve to cause the travel of the material. 75 In order to cool the material and to prevent its oxidation during such cooling, I provide headers 18 located adjacent to the conduit 14 and communicating therewith by a plurality of small apertures 19. The headers 80 are connected to a source of steam or gas supply through the inlet 20. After the material leaves the planishing rolls it immediately enters a reducing atmosphere and is cooled to the point at which no further 85 oxidation will occur. A relatively small quantity of steam or gas will serve to maintain the non-oxidizing atmosphere in the conduit as only sufficient need be employed to prevent the entrance of atmospheric air 90 at the open ends; if, therefore, the steam or gas be supplied at substantially atmospheric pressure, the escape of the fluid from the open ends of the container will only be in proportion to the law as to the diffusion 95 of gases. Therefore a relatively small quantity of the reducing element need be employed. This method has considerable advantage over that which employs the liquid as a cooling medium. 100

I claim:

1. The method of finishing rolled metal products which consists in rolling the products in the usual manner and passing the

rolled product from between the finishing rolls directly into an atmosphere of steam to prevent oxidation thereof while cooling, and enveloping the product in such atmosphere while cooling it to below the point at which oxidation occurs, substantially as described.

2. In apparatus for finishing rolled metal products, the combination with the finishing rolls of an inclosed trough having open ends and arranged to receive the rolled metal as it emerges from said finishing rolls, means for creating a current of elastic fluid within said trough to exclude air and maintain a non-oxidizing atmosphere therein, and means for causing the rolled metal to travel through said trough, substantially as described.

3. In apparatus for finishing rolled metal products, the combination with the finishing rolls of an inclosed trough having open ends and arranged to receive the rolled metal as it emerges from said finishing rolls, means

for creating a current of elastic fluid within said trough to exclude air and maintain a non-oxidizing atmosphere therein, said trough being made in sections and having means between adjoining ends of at least part of said trough sections for causing travel of the metal through said trough, substantially as described. 25

4. Apparatus of the character described, comprising, in combination, planishing rolls, a long open-ended trough mounted at the discharge end of said rolls, a header communicating with said trough by a plurality of small apertures and a source of gaseous fluid connected to said header, substantially as described. 30

Signed at Wheeling, W. Va., this 26 day of September, 1916.

BENJAMIN P. HAZELTINE.

Witnesses:

GIBSON L. CALDWELL,  
J. M. PATTON.